

Sept. 15, 1931.

J. D. CRAMER ET AL

1,823,258

ART OF SPINNING AND TREATING PAPER

Filed Sept. 12, 1929



FIG. 2



FIG. 4



FIG. 3



INVENTOR

J.D. CRAMER  
A.J. ROGERS

BY

*Fisher, Moser & Woodward*

ATTORNEYS

## UNITED STATES PATENT OFFICE

JOSEPH D. CRAMER AND ALBERT J. ROGERS, OF GOSHEN, INDIANA, ASSIGNORS TO THE CHASE BAG COMPANY, OF NEW YORK, N. Y., A CORPORATION OF DELAWARE

## ART OF SPINNING AND TREATING PAPER

Application filed September 12, 1929. Serial No. 392,110.

The present invention relates to the art of spinning and treating paper, and products woven therefrom, and the general object or desire is to produce in a simple and inexpensive way an improved strand of paper having a high tensile strength, water repellent properties and a fast color, from which strong and durable paper bags may be fabricated for shipping and transporting fruits, 10 vegetables and the like in bulk. Thus the invention is predicated on the discovery that many classes of perishable goods, for example, citrus fruits, onions, etc., may be stored or preserved, shipped and transported with 15 advantage and profit in bags made of heavy strands of colored paper coarsely woven together to provide wide open meshes through which the goods may be viewed in their natural state and colors and also thereby exposed to the atmosphere for ventilation, 20 ripening, to prevent mold, etc. Colored strands are desired as given colors or combinations of colors for different classes of goods enhance the appearance thereof when 25 displayed through the meshes of such bags. As an exemplification, citrus fruits such as oranges are more attractively displayed by using red strands spaced apart from cross strands of light tan or natural color, and yellow onions show up to better advantage in 30 bags woven of light yellow strands. The colored strands must be of fast colors inasmuch as they come in contact with edible goods, and are exposed to varying weather 35 conditions, including moisture or water, and the requirements also call for bags capable of holding heavy loads, say one hundred pounds or more of perishable goods. Obviously, therefore, the wall of the bag must 40 be strong and durable and a woven bag made of paper must have warp and woof strands of substantial tensile strength, especially when coarsely woven and widely separated to expose and display the goods. Also, the 45 strength of these strands should not be affected materially when exposed to dampness or a wetting.

In achieving the objects of desire as stated, the treatment accorded the strands in the 50 making thereof, and the steps taken in that

connection, are all factors to be considered. These will now be described in greater detail, reference also being had to the accompanying drawing for a preferred form of apparatus for carrying out and practicing the 55 invention.

Thus, Fig. 1 is an end elevation on a reduced scale, of a machine for spinning paper, and Fig. 2 is a sectional view of parts thereof, on a larger scale, which parts deal with the 60 impregnation of the paper with a coloring solution. Fig. 3 is a side view of a strip of paper partly twisted or spun into a strand, and Fig. 4 is a side view of a small portion of coarsely woven material made of such 65 twisted strands of paper in different colors.

In practicing the invention, a thin flat strip of paper 2, approximately one-eighth or less to one-fourth of an inch in width, is unwound from a roll 3 and wound upon a spool 4 carried by a spinning spindle 5, thereby twisting the strip and producing a tightly spun strand 6. The paper strip passes from roll 3 in a dry state to and underneath a weight 7, which places the strip under tension. 75 Thence the flat strip passes around a reciprocating shaft 8 and over an idler roller 9 to and between a pair of larger rollers 10 and 11, respectively, located directly above the spinning spindle 5. Rollers 10 and 11 function 80 in part to feed the strip onward and in part to apply a liquid compound or spinning solution S containing coloring matter, uniformly to the strip preliminary to twisting or spinning it into a round strand. The solution is contained in a large tank or reservoir 12 and fed by a pipe 14 to an open pan 15 containing a collecting roller 16 which conveys the solution to a distributing roller 17 having contact with the impregnating roller 11 85 around which the paper strip is fed and drawn. The thin paper strip is thoroughly impregnated with the solution and uniformly colored before it is twisted and spun, and the solution used promotes spinning of the 90 paper strip uniformly without breakage and imparts to it water repellent properties and greater tensile strength. Thus a preferred spinning solution consists of an aqueous composition containing soap emulsified with a 100

preservative oil composed of natural glycerides, in any suitable proportions, including a phenol concentrated dye of any desired color.

5      Tightly-twisted strands of paper, so treated, are then woven together, preferably with the strands separated or spaced apart approximately one-eighth of an inch more or less, to provide an open-mesh fabric in  
10     which all the strands may be of the same color, or of different colors. Preferably the warp strands are more firmly or tightly spun and not subjected to a solution containing the phenol dye, therefore stiffer and not quite  
15     as thick or pliable as the colored weft strands which are treated to an emulsified solution containing such a dye. In some cases the warp strands may also be colored. If not, it should be understood that they are treated  
20     nevertheless with the aforesaid solution without a dye, to make them substantially impervious or more repellent to water, and to increase their tensile strength.

25     By adding the phenol dye to the emulsified solution a separate dyeing step or treatment is avoided, the characteristics or properties of the spinning solution somewhat changed, and the coloring of the paper strip made uniform and fast throughout. The steps taken  
30     to produce the colored strands are therefore simple and inexpensive, and the strands so made have a more uniform twist which makes the strand stronger and less apt to break during spinning operations and thereafter when woven into an open mesh fabric and used in a bag as herein described.

What we claim is:

40     A method of producing twisted strands of paper, consisting in spinning a narrow thin strip of paper into a strand and impregnating the strip in the same operation by indirect application with a definite amount of preservative coloring solution having strengthening and water repelling properties.

45     In testimony whereof we affix our signatures.

JOSEPH D. CRAMER.  
ALBERT J. ROGERS.

50

55

60

65